

May 7, 1974

G. STEVEN

3,809,541

VANADIUM-CONTAINING TOOL STEEL ARTICLE

Filed Oct. 24, 1972

2 Sheets-Sheet 1



FIG. 1



FIG. 2



FIG. 3

May 7, 1974

G. STEVEN

3,809,541

VANADIUM-CONTAINING TOOL STEEL ARTICLE

Filed Oct. 24, 1972

2 Sheets-Sheet 2



*FIG. 4*



*FIG. 5*

**1**

3,809,541

**VANADIUM-CONTAINING TOOL STEEL ARTICLE**Gary Steven, 444 Royce Ave., Pittsburgh, Pa. 15216  
Filed Oct. 24, 1972, Ser. No. 300,094

Int. Cl. C22c 39/14

U.S. Cl. 29—192

2 Claims

**ABSTRACT OF THE DISCLOSURE**

A vanadium-containing tool steel and article compacted from particles thereof and a method for producing said article from a prealloyed powdered charge of the alloy consisting essentially of, in weight percent, carbon 1.5 to 1.6, chromium 3.5 to 4.5, vanadium 2.5 to 3.5, tungsten 9 to 11, molybdenum 4.5 to 5.5, cobalt 8.0 to 12.5, manganese up to 1, silicon up to 1, nitrogen .02 to .08 and balance iron; the article is characterized by the combination of hardness and toughness making it desirable for cutting tool applications.

In the use of tool steel articles for high-speed cutting tool applications, a good combination of wear resistance and high toughness is necessary for obtaining prolonged tool life. Wear resistance is promoted by high hardness and, particularly, by high MC-type (vanadium) carbide content of the tool steel. On the other hand, toughness—commonly measured in terms of impact strength—also contributes to tool life in that, particularly in intermittent cutting applications, the tool is able to withstand repeated impacts during cutting without breaking. But the combination of high wear resistance and high toughness is difficult to achieve, because of the MC-type carbide content is increased by the necessary changes in the composition of the steel, the toughness or impact resistance of the steel decreases.

It is accordingly the primary object of this invention to provide a tool steel that overcomes the above-described, prior-art problem of achieving both of the desired properties of wear resistance and toughness in combination.

This and other objects of the invention, as well as a complete understanding thereof, may be obtained from the following description, specific examples and drawings, in which:

FIG. 1 is a graph showing the amount of MC-type (vanadium) carbide in the as-hardened structure of conventional high-speed steels AISI M1, M4 and T15;

FIG. 2 is a similar graph showing the effect of MC-type (vanadium) carbide contents on the toughness of these three conventional steels when heat treated to a hardness of  $R_c$  65;

FIG. 3 is a graph showing the effect of the MC-type (vanadium) carbide contents of these three conventional steels on the wear resistance when heat treated to a hardness of  $R_c$  64;

FIG. 4 is a photomicrograph of a steel compact in accordance with the present invention showing the carbide size and distribution thereof at a magnification of 1000 $\times$ ; and

FIG. 5 is a photomicrograph showing the prior austenite grain size of the compact of FIG. 4 at a magnification of 1000 $\times$ .

The tool steel of the invention consists essentially of, in weight percent, carbon 1.5 to 1.6, chromium 3.5 to 4.5, vanadium 2.5 to 3.5, tungsten 9 to 11, molybdenum 4.5 to 5.5, cobalt 8.0 to 12.5, manganese up to 1, silicon up to 1, nitrogen .02 to .08 and balance iron. In accordance with the invention, this steel is used in the form of powder of about minus 16 mesh U.S. Standard. This powder is placed in a metal container, which is gas tight.

**2**

The container is heated to an elevated temperature in excess of about 2000° F. and during the initial stages of heating its interior is pumped to a low pressure whereupon the gaseous reaction products and principally those resulting from the reaction of carbon and oxygen are removed from the interior of the container, which operation is termed as "outgassing." Thereafter and upon removal of the gaseous reaction products, the container is heated to or above the desired compacting temperature, which is in excess of about 2130° F., and with the container sealed against the atmosphere it is transferred to a compacting apparatus. Compacting may be achieved by use of a mechanical apparatus wherein the sealed container is placed in a die and a ram is inserted therein to compact the container and charge. Alternately, the container may be placed in a fluid-pressure vessel, commonly termed an "autoclave," wherein a fluid pressure medium, such as nitrogen gas, may be employed for compacting. In any event, however, compacting is completed to a density greater than about 95% of theoretical prior to the charge cooling to a temperature below about 1900° F. If desired, compacting to this density may be achieved by a plurality of separate compacting operations, and the powder charge may be precompacted to a low density, e.g. 60%, prior to outgassing. After compacting, conventional machining or forming operations incident to cutting tool manufacture may be performed.

It was heretofore believed, as may be seen from a study of FIGS. 1, 2 and 3 of the drawings, that as the vanadium content and correspondingly the carbon content of the alloys of this type are increased to increase the MC-type (vanadium) carbide content of the alloy its wear resistance is increased while its toughness, as a function of impact value, is decreased. With the present invention it has been found, however, that if carbon is maintained within the range of 1.5 to 1.6% in combination with a vanadium content of 2.5 to 3.5%, as will be specifically explained and shown hereinafter, high wear resistance may be achieved without an attendant decrease in toughness.

In the heat treating of articles in accordance with the invention, the articles are austenitized at a temperature on the order of 2170° F. and then hardened during cooling. The austenitizing step involves heating to a temperature sufficient to dissolve, to a considerable extent, the carbide phases present in the microstructure of the steel. After quenching from the austenitizing temperature, the article is subjected to reheating at a lower temperature in which case carbide-forming elements, e.g. vanadium, tungsten and molybdenum, are precipitated in the form of fine carbides. This, of course, produces the secondary hardening necessary for high-speed cutting applications. During austenitizing, much of the carbon is dissolved in the austenite, which upon cooling transforms to a hard carbon-containing martensite. The carbide-forming elements remain in solution in the martensite. Subsequently, however, the carbide-forming elements during tempering combine with the carbon in the steel and form carbides. It is this carbide precipitation which produces the desired secondary hardening.

As above stated, the restricted combination of carbon and vanadium in the alloy achieves the result of a good combination of wear resistance and toughness. In addition, the cobalt present in the alloy contributes to the retention of hardness at high temperature, to which the alloy articles are subjected during high-speed cutting use. Nitrogen is necessary to achieve a desired fine carbide distribution. Both molybdenum and tungsten within the recited limits are necessary to obtain sufficient heat resistance for operation of a cutting tool at high speeds.

TABLE I

| Steel designation | Internal code | Composition, weight percent |     |      |      |     |     |      |      |     |      |     |
|-------------------|---------------|-----------------------------|-----|------|------|-----|-----|------|------|-----|------|-----|
|                   |               | C                           | Mn  | S    | P    | Si  | Cr  | V    | W    | Mo  | Co   | N   |
| A-----            | 391-77        | 1.42                        | .26 | .031 | .013 | .34 | 3.8 | 3.0  | 9.5  | 5.2 | 11.8 | .05 |
| B-----            | 391-84        | 1.56                        | .26 | .031 | .013 | .34 | 3.8 | 3.0  | 9.5  | 5.2 | 11.8 | .05 |
| C-----            | P65430        | 1.65                        | .33 | .010 | .010 | .30 | 3.7 | 3.1  | 10.0 | 5.2 | 12.3 | .03 |
| D-----            | P65056        | 1.15                        | .33 | .013 | .010 | .36 | 3.7 | 1.25 | 10.2 | 5.2 | 12.1 | .03 |

To demonstrate the present invention, and by way of specific examples thereof, samples of the steels designated as A, B, C and D with the compositions listed in Table I were produced. Steel B is within the composition limits of the present invention; whereas, steels A and D have carbon contents below that of the steel in accordance with the present invention, and steel C has a carbon content higher than that of the steel of the present invention.

More specifically, powdered charges of steels A, B, C and D of Table I were made by conventional gas atomizing and screened to a size consist of minus 16 mesh U.S. Standard. Each of the particle charges of steels A, B, C and D were processed in the following manner. A particle charge of A and B was placed in a mild-steel cylinder about 6" length and having a diameter of 5½". The particle charge of C and D was filled into a cylinder about 48" length and having a diameter of about 11". The particle-filled container was heated to a temperature of about 2100° F. for about 5 hours, and during the early stages of heating the interior of the container was connected to a vacuum pump which was used to remove the gaseous reaction products from the container. The container and charge were compacted to achieve a density of about 99% of theoretical by the use of an isostatic compaction pressure of 15,000 p.s.i. in a gas pressure vessel with nitrogen being the gaseous pressure medium employed.

After compacting, the compacted article was forged into 1" square bars. The bars were then austenitized at 2160° F. for 2 minutes and then oil quenched. Microscopic examination of these bars showed a uniform dispersion of carbides in an iron-rich alloy matrix, and further that the carbide phase particles were predominantly less than 3 microns in size.

TABLE II

| Tool material               | Tool hardness (R <sub>c</sub> ) | Average tool life in—     |                                          |                       |
|-----------------------------|---------------------------------|---------------------------|------------------------------------------|-----------------------|
|                             |                                 | Continuous cutting (min.) | Intermittent cutting (number of impacts) | Average tool life in— |
| Steel A, 1.42% C-----       | 68.5                            | 39                        | 3,110                                    |                       |
| Steel B, 1.56% C-----       | 69.5                            | 40                        | 5,080                                    |                       |
| Steel C, 1.65% C-----       | 70.0                            | 65                        | 2,260                                    |                       |
| Steel D, 1.15% C-----       | 68.5                            | 30                        | 2,810                                    |                       |
| AISI type T15, 1.50% C----- | 67.0                            | 21                        | 1,700                                    |                       |

To test the tool performance, ½" square tool bits were prepared from forged bars of steels A, B, C and D; the tool geometry was: 3°, 6°, 10°, 10°, 10°, 0.030" nose radius. These tool bits were heat treated by austenitizing at 2160° F. for 2 minutes, quenching into a salt bath at 1100° F., holding for 5 minutes, air cooling to ambient temperature, and tempering at 1025° F. for 2+2+2 hours. The resulting hardnesses are included in Table II. The microstructure of steel B is shown in FIGS. 4 and 5.

For comparison, ½" square tool bits with the same geometry as the tools produced from the bars of steels A, B, C and D were prepared from commercial stock of the well-known AISI Type T15 high-performance high-

speed tool steel and heat treated in accordance with the recommended commercial practice to 67 R<sub>c</sub> hardness. First, all tool bits were tested for performance in continuous lathe turning of an AISI H13 workpiece heat treated to 300 BHN. The cutting speed was 55 s.f.p.m.; feed—0.010" per revolution; depth-of-cut 1/16"; coolant—none; test end-point 0.015" flank wear. The results of Table II show that, as expected, tool life was increased with increased vanadium carbide content and hardness. Steels A, B, and C as a group were distinctly superior to steel D as well as to AISI Type T15 high-performance high-speed tool steel. Within the A, B, C group, tool life increased from steel A to steel B to steel C, i.e., in the order of the increasing carbon or vanadium carbide contents, as expected.

Then intermittent cut-lathe turning tests were conducted using a four-slotted AISI H13 workpiece heat treated to 300 BHN. The speed was 50 s.f.p.m.; feed 0.010" per revolution; depth-of-cut 1/16"; coolant—none; test end-point 0.015" flank wear. At least three tests were run on each tool material. The results of Table II revealed an unexpected result—the intermittent-cut tool life of steel B (containing 1.56% carbon) was distinctly superior to those obtained with steels A (lower carbon) and C (higher carbon) as well as steel D (lower carbon and lower vanadium) and AISI Type T15, which is well known as a high-performance high-speed steel. A definite criticality of the carbon content of the inventive steel in the range of 1.50 to 1.60% is indicated. This finding is even more surprising when the higher hardness of steel B (R<sub>c</sub> 69.5) in comparison to steel A (R<sub>c</sub> 68.5) and steel D (R<sub>c</sub> 68.5) is taken into consideration. As explained hereinabove, at this higher hardness, one would expect that the toughness of the tool bit of steel B, as demonstrated by intermittent cut tool life, would decrease.

What is claimed is:

1. A fully dense, tool-steel, powder-metallurgy compacted article produced from prealloyed tool-steel powder consisting essentially of, in weight percent, carbon 1.5 to 1.6, chromium 3.5 to 4.5, vanadium 2.5 to 3.5, tungsten 9 to 11, molybdenum 4.5 to 5.5, cobalt 8.0 to 12.5, manganese up to 1, silicon up to 1, nitrogen .02 to .08 and balance iron.

2. The article of claim 1 having a substantially uniform carbide dispersion with the carbide particles predominantly less than three microns in size.

#### References Cited

#### UNITED STATES PATENTS

|           |         |          |          |
|-----------|---------|----------|----------|
| 1,206,834 | 12/1916 | Furness  | 75—126 E |
| 1,876,725 | 9/1932  | Mitchell | 75—126 E |
| 1,998,956 | 4/1935  | Emmons   | 75—126 E |
| 2,590,835 | 4/1952  | Kirkby   | 75—126 E |

HYLAND BIZOT, Primary Examiner

U.S. CL. X.R.

75—126 C, 126 V, 126 H, 126 A